

# United States Patent Office

3,352,787

Patented Nov. 14, 1967

1

3,352,787

INHIBITION OF PLASTIC CRAZING  
Charles M. Bodach, Morton Grove, Ill., assignor, by  
mesne assignments, to W. R. Grace & Co., New York,  
N.Y., a corporation of Connecticut  
No Drawing. Filed Dec. 11, 1963, Ser. No. 329,878  
10 Claims. (Cl. 252—108)

The present invention relates to improvements in the field of cleaners, and more specifically, to the cleaning of resinous materials which are subject to crazing.

Specifications for cleaning compounds, whether liquid or powder, frequently require that the cleaning material provide no deleterious effect on plastics. For example, government specifications for cleaning aircraft surfaces require that the cleaner shall be nonreactive with respect to "Plexiglas" surfaces such as those of the windshields of aircraft. In fact, the government has issued a specific stress-crazing test which a material must meet in order to be acceptable.

In formulating cleaners for various purposes, including the cleaning of transparent acrylic base plastics, it would be highly desirable to include a significant amount of a non-ionic surfactant because of the excellent detergent properties of the non-ionic materials, and their relatively low cost. However, it was found that the use of many non-ionic surfactants created a crazing problem when applied to a stressed acrylic base plastic material.

I have now found that the crazing properties of these non-ionic surfactants can be overcome by the inclusion of ionic (anionic or cationic) surfactants in the same composition. These materials have the ability to not only inhibit the crazing tendencies characteristic of the non-ionic surfactant but also improve the detergency.

An object of the present invention is to provide an improved composition for cleaning stressed acrylic base materials utilizing non-ionic surfactants without providing crazing of the surfaces.

A further object of the invention is to provide an improved cleaning composition adapted for cleaning transparent plastic surfaces including relatively large amounts of an inexpensive, non-ionic surfactant.

Still another object of the invention is to provide a method for cleaning stressed acrylic base surfaces without presenting the problem of crazing.

The compositions and method of the present invention are applicable to various physical forms of acrylic base plastics, including sheet material, filaments, fabrics and the like.

The cleaning compositions and method of the present invention are applicable to all types of light transmitting acrylic base polymers including polyacrylates and polymethacrylates. The invention has particular utility in connection with the cleaning of polymethyl methacrylate "Plexiglas," a commercially available material which usually has a light transmission of 91 to 92%, a refractive index of about 1.49, a density of about 1.18, and a tensile strength of 7,000 to 9,000 p.s.i.

Certain non-ionic surfactant materials pose particularly troublesome crazing problems when applied to light transmitting, stressed acrylic based polymers. Among these are the materials known commercially as "Triton" which are non-ionic surface active agents prepared by the reaction of t-octylphenol or nonylphenol with ethylene oxide. These products are commercially described as alkyl aryl polyether alcohols or alkyl phenol ethers of polyethylene glycol. The number of ethylene oxide groups in the molecule may vary from about 1 to 30 and typically may contain 9 to 10 ethylene oxide groups ("Triton X-100"), or 12 to 13 ethylene oxide groups ("Triton X-102").

Another series of non-ionic surfactants which present

2

crazing problems are those known commercially as "Igepal," these being polyoxyethylated nonylphenols produced by the chemical reaction of nonylphenol with varying amounts of ethylene oxide ranging from 1½ to 30 moles of ethylene oxide per mole of nonylphenol. The corresponding ethylene oxide contents in the final product range from about 23 to 86%.

Still another class of materials which exhibit crazing problems in this connection are certain "Pluronics" which are block polymers consisting of a polyoxypropylene hydrophobic base and hydrophilic polyoxyethylene chains attached thereto.

As far as I have been able to determine, any anionic surfactant or any cationic surfactant material, when added in proper amounts is capable of neutralizing the tendency of the non-ionic materials to cause crazing of the light transmitting acrylic surface. Derivatives of carboxylic acids, including rosin and tall oil acids, are useful as are sulphuric esters derived from olefins and alcohols. Alkane sulfonates with and without intermediate linkages can also be employed. Mahogany and petroleum sulfonates, as well as other anionic surfactants such as phosphorus compounds, lignin derivatives, and the like can also be used. Particularly good results are obtained through the use of an alkyl aryl sulfonate (in the form of a sodium salt), the alkyl group containing from about 6 to 20 carbon atoms.

Similarly, the cationic surfactants may be either non-quaternary material such as nitriles, amines, or other 30 nitrogen bases, as well as the better known quaternary cationic materials.

Specific examples of compositions embodying the improvements of the present invention will be found in a succeeding portion of this description. However, it should be recognized that the usable anionic and cationic surfactants are not limited by the examples, but can be any of the materials which fall into these designations. The invention contemplates that two or more anionic agents or two or more cationic agents can be used simultaneously. A more comprehensive discussion of anionic surfactants, and methods for their preparation will be found in the book, "Surface Active Agents and Detergents," volume 2, by Schwartz, Perry and Berch (Interscience Publishers, 1958), pages 25 to 102. A similar discussion of cationic surfactants will be found in the same work, at pages 103 to 119.

While the proportions between the non-ionic and the 50 ionic surfactant will vary over a wide range depending on the particular composition, it has been found that for most purposes, the amount of added anionic or cationic agent should be from  $\frac{1}{20}$  to 5 times the amount of non-ionic surfactant present, and preferably from  $\frac{1}{5}$  to 2 times. It should be recognized, of course, that any cleaning composition embodying the combination of non-ionic and ionic surfactants may also include alkali metal tripolyphosphates and other polyphosphates, builders, sequestering agents, and the like.

The government approved test for stress crazing of acrylic base plastics requires that three specimens of sheet acrylic plastic be annealed by suspending in an oven maintained at  $90^\circ \pm 2^\circ$  C. for 2 hours. At the end of the annealing period, the temperature of the specimens is reduced to room temperature at a maximum rate of  $27^\circ \pm 5^\circ$  C. per hour. The annealed specimens are conditioned at room temperature for at least 7 days before use. The three specimens are then set up in cantilever fashion and carefully stressed to 3,000 lbs. per sq. in. outer fiber stress. After 10 minutes, the specimens are examined to insure that no crazing has occurred prior to the application of the cleaning compound. When the specimens are still under stress, an absorbent cotton swatch approximately  $\frac{3}{4}$  inch square is placed on the tension side of the

specimen, directly over the fulcrum on which it is mounted. The cleaning compound is carefully applied to the cotton swatch and the swatch is kept wet by additional applications as necessary. After 24 hours and while the specimen is still under stress, the cotton swatch is removed and the specimens are examined for crazing, cracking, or other attack. The load is then removed and the specimens are rinsed with tap water and re-examined for crazing, cracking, or other attack.

Using this standard test, the following compositions, all containing a non-ionic surfactant and various amounts of other materials were found to cause crazing:

|     | Solution                                                                                                                   | Percent                | Results |
|-----|----------------------------------------------------------------------------------------------------------------------------|------------------------|---------|
| 1.  | Water<br>"Igepal CO 880" (30 ethylene oxide groups).<br>"Triton N-128" (12-13 ethylene oxide groups).                      | 90<br>5                | Crazed. |
| 2.  | Water<br>"Triton X-102" (12-13 ethylene oxide groups).                                                                     | 95<br>5                | Do.     |
| 3.  | Water<br>"Triton N-128"                                                                                                    | 95<br>5                | Do.     |
| 4.  | Water<br>"Igepal CO 730" (15 ethylene oxide groups).                                                                       | 95<br>5                | Do.     |
| 5.  | Water<br>"Triton Cf-10"                                                                                                    | 95<br>5                | Do.     |
| 6.  | Water<br>"Pluronic L-44"                                                                                                   | 95<br>5                | Do.     |
| 7.  | Water<br>"Pluronic F-75"                                                                                                   | 95<br>5                | Do.     |
| 8.  | Water<br>"Triton X-165" (16 ethylene oxide groups).                                                                        | 95<br>5                | Do.     |
| 9.  | Water<br>"Triton X-205" (20 ethylene oxide groups).                                                                        | 95<br>5                | Do.     |
| 10. | Water<br>"Triton X-305" (30 ethylene oxide groups).                                                                        | 95<br>5                | Do.     |
| 11. | Water<br>"Igepal CO 850" (20 ethylene oxide groups).                                                                       | 95<br>5                | Do.     |
| 12. | Water<br>Tetrapotassium pyrophosphate (TKPP).<br>Sodium metasilicate pentahydrate.<br>Sodium gluconate.<br>"Triton X-102". | 85<br>3<br>5<br>2<br>5 | Do.     |
| 13. | Water<br>TKPP.<br>Sodium metasilicate pentahydrate.<br>Sodium gluconate.<br>"Triton X-102".<br>Butyl Cellosolve.           | 83<br>5<br>5<br>2<br>5 | Do.     |
| 14. | Water<br>TKPP.<br>Sodium metasilicate pentahydrate.<br>"Triton X-165".                                                     | 85<br>3<br>5<br>7      | Do.     |
| 15. | #2 fuel oil<br>"Triton X-45" (5 ethylene oxide groups).                                                                    | 95<br>5                | Do.     |

Inclusion of varying amounts of anionic and cationic surfactants in these compositions eliminated the crazing problem, as evidenced from the following examples:

|     | Solution                                                                                                      | Percent          | Results     |
|-----|---------------------------------------------------------------------------------------------------------------|------------------|-------------|
| 16. | Water<br>"Triton X-102".<br>"Dresinate TX" (sodium salt of tall oil).                                         | 95<br>2<br>3     | No crazing. |
| 17. | Water<br>"Triton X-102".<br>"Ultrawet DS" (sodium salt of alkyl benzene sulfonate).                           | 95<br>2<br>3     | Do.         |
| 18. | Water<br>"Triton X-100".<br>"Hyamine 1622" (para disobutyl phenoxy ethoxy dimethyl benzyl ammonium chloride). | 92.5<br>5<br>2.5 | Do.         |

|     | Solution                                                                                                                          | Percent                                 | Results |
|-----|-----------------------------------------------------------------------------------------------------------------------------------|-----------------------------------------|---------|
| 19. | Water<br>"Triton X-100".<br>"Duponol ME" (Lauryl alcohol sulfate).                                                                | 92.5<br>5<br>2.5                        | Do.     |
| 20. | Water<br>"Triton X-100".<br>Sodium xylene sulfonate.                                                                              | 92.5<br>5<br>2.5                        | Do.     |
| 21. | Water<br>"Triton X-100".<br>"Marasperse N" (sodium lignosulfonate).                                                               | 92.5<br>5<br>2.5                        | Do.     |
| 22. | Water<br>TKPP.<br>Sodium metasilicate pentahydrate.<br>"Ultrawet DS".<br>"Triton X-165".                                          | 85<br>3<br>5<br>2<br>5                  | Do.     |
| 23. | Water<br>TKPP.<br>Sodium metasilicate pentahydrate.<br>"Ultrawet DS".<br>"Triton X-102".                                          | 85<br>1<br>5<br>3<br>6                  | Do.     |
| 24. | Water<br>TKPP.<br>Sodium metasilicate pentahydrate.<br>"Ultrawet DS".<br>"Triton X-100".                                          | 85<br>1<br>5<br>3<br>6                  | Do.     |
| 25. | Water<br>Tetrasodium pyrophosphate (TSPP).<br>Sodium metasilicate pentahydrate.<br>"Dresinate T".<br>"Triton X-102".              | 85.5<br>1.0<br>5.0<br>2.0<br>6.5        | Do.     |
| 26. | Water<br>TSPP.<br>Sodium metasilicate pentahydrate.<br>"Dresinate TX".<br>Sodium gluconate.<br>"Triton X-100".                    | 85.5<br>1.0<br>5.0<br>2.0<br>1.0<br>5.5 | Do.     |
| 27. | Water<br>Sodium tripolyphosphate.<br>Sodium metasilicate pentahydrate.<br>"Dresinate TX".<br>Sodium gluconate.<br>"Triton X-102". | 85.0<br>1.0<br>5.0<br>1.5<br>2.5<br>5.0 | Do.     |
| 28. | Water<br>TKPP.<br>Sodium metasilicate pentahydrate.<br>Sodium gluconate.<br>"Triton X-102".                                       | 83<br>1.0<br>5.0<br>2.0<br>5.0          | Do.     |
| 29. | Water<br>TKPP.<br>Sodium metasilicate pentahydrate.<br>Sodium gluconate.<br>"Triton X-102".                                       | 83<br>1.0<br>5.0<br>2.0<br>5.0          | Do.     |
| 30. | Water<br>TSPP.<br>Sodium metasilicate pentahydrate.<br>"Dresinate TX".<br>Sodium gluconate.<br>"Triton X-102".                    | 85.5<br>1.0<br>5.0<br>2.0<br>1.0<br>5.5 | Do.     |

45 By comparison of Example 2 with Examples 16 and 17, it will be noted that the substitution of the anionic agent for the corresponding amount of non-ionic agent entirely eliminated the crazing. Similarly, by comparing Example 14 with Example 22 it will be seen that the substitution of 50 a portion of the non-ionic surfactant with an anionic surfactant, all other things being constant, eliminated the crazing problem.

55 From the foregoing, it will be seen that compositions of the present invention eliminate the crazing problem which occurs when many non-ionic surfactants are applied in solution over a surface of a stressed, light transmitting acrylic base resin. It should also be noted that this crazing inhibition persists even though the compositions may also contain diverse materials such as phosphates, silicates, and salts of organic acids.

60 It should also be evident that various modifications can be made to the described embodiments without departing from the scope of the present invention.

I claim as my invention:

65 1. The method of washing a stressed acrylic base sheet which comprises applying thereto an aqueous solution of a polyethoxylated non-ionic surfactant which normally exhibits crazing properties when applied to stressed acrylic base sheets and from  $\frac{1}{20}$  to 5 times the weight of the non-ionic surfactant, of a water-soluble ionic surfactant selected from the group consisting of alkyl benzene sulfonates having from 6 to 20 carbons in the alkyl group, xylene sulfonates, lignosulfonates, tall oil salts, petroleum sulfonates, lauryl alcohol sulfate, and diisobutyl phenoxy ethoxy dimethyl benzyl ammonium chloride.

2. The method of claim 1 wherein the non-ionic surfactant is a polyethoxylated alkyl phenol having from 8 to 9 carbons in the alkyl group and from 1 to 30 ethoxy groups.

3. The method of claim 1 wherein the non-ionic surfactant is a polyoxyethylene-polyoxypropylene copolymer.

4. The method of claim 1 wherein the ionic surfactant is an alkyl-benzene sulfonate having from 6 to 20 carbons in the alkyl group.

5. The method of claim 1 wherein the ionic surfactant is a sodium lignosulfonate.

6. The method of claim 1 wherein the ionic surfactant is a sodium salt of tall oil.

7. The method of claim 1 wherein the ionic surfactant is a petroleum sulfonate.

8. The method of claim 1 wherein the ionic surfactant is lauryl alcohol sulfate.

9. The method of claim 1 wherein the ionic surfactant is diisobutyl phenoxy ethoxy dimethyl benzyl ammonium chloride.

10. The method of claim 1 wherein said aqueous solution contains about one weight percent sodium tripolyphosphate, about 5 weight percent sodium metasilicate, from about 1.5 to 2 weight percent of sodium salts of tall oil, from about 1 to 2.5 weight percent sodium gluconate, and from about 5 to 5.5 weight percent of a poly-

5

6

ethoxylated alkyl phenol having from 8 to 9 carbons in the alkyl group and from 12 to 13 ethoxy groups.

#### References Cited

##### UNITED STATES PATENTS

|           |         |           |       |         |
|-----------|---------|-----------|-------|---------|
| 2,292,097 | 8/1942  | Vollmer   | ----- | 106—13  |
| 2,353,978 | 7/1944  | Weber     | ----- | 106—13  |
| 2,372,171 | 3/1945  | Bennett   | ----- | 106—13  |
| 2,726,962 | 12/1955 | Iorio     | ----- | 106—13  |
| 2,878,188 | 3/1959  | Callahan  | ----- | 252—136 |
| 2,948,625 | 8/1960  | MacKenzie | ----- | 106—13  |

##### FOREIGN PATENTS

|    |         |         |                |  |
|----|---------|---------|----------------|--|
| 15 | 654,005 | 12/1962 | Canada,        |  |
|    | 808,805 | 2/1959  | Great Britain. |  |

##### OTHER REFERENCES

Surface Active Agents and Detergents, vol. II, Schwartz et al., Interscience Publishers, Inc., N.Y. 1958, pp. 210, 32, 33, 101.

LEON D. ROSDOL, *Primary Examiner.*

SAMUEL H. BLECH, *Examiner.*

S. E. SCHNEIDER, *Assistant Examiner.*

25